

1,194,589.

N. BARRY.

PROCESS OF MAKING STEEL PULLEYS.

APPLICATION FILED JULY 30, 1915.

Patented Aug. 15, 1916.

2 SHEETS—SHEET 1.



Inventor

Nicholas Barry

By Dowell & Dowell

Attorneys

Witnesses

B. M. Offutt,

W. Wallace Nairn Jr.

N. BARRY,  
PROCESS OF MAKING STEEL PULLEYS,  
APPLICATION FILED JULY 30, 1915.

1,194,589.

Patented Aug. 15, 1916.

2 SHEETS—SHEET 2.



Inventor

Witnessed  
R. M. Coffey

W. W. Wallace, Jr.

Nicholas Barry  
By  
Fowell & Fowell  
Attorneys

# UNITED STATES PATENT OFFICE.

NICHOLAS BARRY, OF MUSCATINE, IOWA, ASSIGNOR TO BARRY COMPANY, OF MUSCATINE, IOWA, A CORPORATION OF IOWA.

## PROCESS OF MAKING STEEL PULLEYS.

1,194,589.

Specification of Letters Patent. Patented Aug. 15, 1916.

Application filed July 30, 1915. Serial No. 42,737.

To all whom it may concern:

Be it known that I, NICHOLAS BARRY, a citizen of the United States, residing at Muscatine, in the county of Muscatine and State of Iowa, have invented certain new and useful Improvements in Processes of Making Steel Pulleys; and I hereby declare that the following is a full, clear, and exact description thereof, reference being had to the accompanying drawings, which form part of this specification.

This invention relates to sheet metal pulleys and the like, and has particular reference to the manufacture of "split pulleys" out of sheet metal; and its object is to enable such pulleys to be substantially made of light sheet metal as compared with what it has heretofore been necessary to use for pulleys of a given size and strength. The present invention resides in the novel process of making sheet metal pulleys, which process consists essentially in first forming the several members of the pulley, (such as the hub, spokes and rim members of the pulley) out of separate pieces of sheet metal; second assembling the members together to form a pulley or split-pulley section and rigidly connecting the members, preferably by electric welds, so as to hold them in proper relative position and close together; and third dipping such pulley or split-pulley section as a whole, into a bath of molten metal or applying molten metal thereto in such manner and quantity as will fill all the crevices between such members at the points adjacent the connections or welds uniting same, and sweat or solder the connected members together.

Pulleys made in accordance with this invention have substantially all of the advantages of lightness possessed by the best wooden split pulleys of equal diameter and width, and also have all the advantages of strength possessed by the best metal pulleys of equal diameter and width heretofore made.

To impart a clear understanding of the present invention, I will describe the same as used in making split sheet metal pulleys, and the accompanying drawings illustrate a practical pulley manufactured in accordance with the present invention.

In said drawings: Figure 1 represents a face view of a complete split pulley; Fig. 2 is a sectional view thereof; Fig. 3 is an en-

larged inner face view of one split pulley section; Fig. 4 is an enlarged sectional view indicating how the stamped sheet metal members of the pulley are assembled and connected by electric welds; and Fig. 5 is a similar view showing the process of construction completed.

Preferably the pulley is "split", and formed of similar opposite sections. The opposite sections of the pulley are constructed alike, and may be united together around a shaft by suitable clamps, not shown, in the well known manner. Each section comprises a rim portion 1, having beads 1<sup>a</sup> on its sides; each bead having an internal end flange 1<sup>c</sup> which lies against the inner face of the rim 1. Each rim portion is stiffened by a central internal U-shaped metal reinforce 2, to which are connected the outer ends of tubular sheet metal spokes 3, and the inner ends of said spokes are connected to a hub formed of similar opposite sheet metal members 5. Each rim section of the pulley is provided with sheet metal end plates 7. Each rim member 1, reinforce 2, spoke 3, hub member 5 and plate 7 is preferably stamped or pressed out of sheet metal. All the parts are preferably shaped as illustrated in the drawings, but may be of other forms if desired.

In carrying out my invention the members are assembled in proper relative position and permanently united by suitable means. I prefer to unite the members by electric welding, spot welds being indicated at *w* in Figs. 4 and 5 of the drawings. Where the members are united there will be some slight crevices or spaces left between the opposed portions of the united parts, as indicated at *c* in Fig. 4. But after the members have been assembled and united as described the pulley or pulley section, as a unit is dipped into a bath of molten metal, preferably composed of tin and lead or other metals, which molten metal flows into and fills all the crevices between the adjacent members, as indicated at *c* in Fig. 5, and also adheres to and solders or combines the opposed surfaces of the connected members, and the exterior surfaces of the members will also be coated with such metal as indicated by the heavy lines *C* in Fig. 5.

In practically using my process I preferably stamp or press the various pulley members out of pickled sheet metal, that is metal

22

sheets that have been cleansed in a weak sulfuric acid solution or other suitable bath. The members are then assembled and united, preferably by spot welding, as stated to 5 form a pulley or pulley section. Then the pulley or pulley section is dipped in a pickling bath to cleanse the surfaces thereof from grease and dirt. Then the pulley or pulley section is dipped or immersed in a 10 bath of molten metal, as stated, and should be left in this bath long enough to heat the members of the sections to approximately the same temperature as the molten bath, which will cause the molten metal to coat the 15 surfaces of the pulley and fill all the slight crevices between the connected parts thereof; I have found that these crevices will be filled because the molten metal or solder has a tendency to flow over and cover all the 20 metal surface with which it comes in contact, and over all exposed surfaces. Such dipping in molten solder or tin insures coating of all the exterior surfaces of the pulley and the filling up of all the crevices between 25 the members thereof, so that the members become rigidly united and bonded or soldered together, and the pulley becomes practically as unitary and homogeneous as if made in one piece.

30 Light metal pulleys which can take the place of wooden pulleys and be as easily handled have been greatly desired, and I have succeeded in making such a pulley by the described process the metal or solder 35 forming an absolutely permanent connection between the members. Light pulleys, require less power to operate, but they must be able to withstand the working strains and in order to insure this I dip the pulleys in 40 molten solder or tin not merely to protect the metal from oxidization, but principally to fill all the crevices or joints between the spot welds and firmly and permanently unite the members; and this filling of all crevices 45 by the metal prevents weakening of the welds or other fastenings.

As stated, after the pulley sections are assembled they are preferably dipped in molten tin, or other suitable metal or composition of metal, which fills the crevices at the 50 bends and joints and renders the surface of the pulley smooth and practically solders the parts together and protects the parts against rust, and any slight crevices between 55 opposed unwelded portions will be filled by the molten metal in the soldering process, thus producing close joints and preventing looseness of parts. I have found by actual test that this dipping in metal increases the 60 strength of the pulley about thirty per cent. Such pulleys are especially useful where exposed to dampness or to action of gases

which would be detrimental to ordinary pulleys. Sheet metal pulleys constructed in accordance with my process are equivalent in 65 strength to an integral metal pulley, and can be made as light as a wooden pulley of the same size. The pulleys may be even lighter than wooden pulleys for in actual practice a twenty-four inch pulley four inch 70 face made in accordance with my invention will weigh about sixteen pounds, whereas a wooden pulley of the same size would weigh about thirty pounds. By this process of manufacture I am able to make pulleys out 75 of much thinner metal than would otherwise be practical. If the same pulley was made without the step of dipping, soldering or tinning, the members thereof—because of their lightness—would in use vibrate between the welds and in a short time cause 80 the welds to crystallize and the pulley would go to pieces; but by dipping or sweating the pulleys in hot metal as described the fluid metal fills all the crevices or cracks in the 85 joints and between the welds and practically amalgamates the several pieces and binds them solidly together as one piece and eliminates vibration and consequently prevents weakening of the welds. The soldering or 90 tinning is not merely intended to prevent rust or to enhance the appearance of the pulley, but primarily to consolidate the pieces by filling all the loose joints or crevices with metal which becomes practically an integral 95 part of the metal of the pulley and renders same practically homogeneous, stiff and strong.

In the specification and claim the expression "dipping the molten metal" is intended 100 to cover dipping the pulley sections in molten tin or other suitable metal or composition of metals, or so applying such hot metal to the parts as will effectively close the joints and crevices between the connected pieces 105 and firmly bond them together thus making the parts practically homogeneous and capable of withstanding great strain without injury and contributing most materially to the durability and serviceability of the pulley. 110

What I claim is:

The herein described process of making sheet metal pulleys consisting in separately forming the several members thereof out of sheet metal; then assembling and rigidly 115 connecting such members by electric welds; then dipping the whole in molten metal to close all the crevices between the united parts of the members and around the welds and solidly solder the parts together, substantially as described.

In testimony that I claim the foregoing as my own, I affix my signature.

NICHOLAS BARRY.